

B. C. LAUTH.

METHOD FOR MAKING A MATERIAL HAVING THE GENERAL PROPERTIES OF WROUGHT IRON.  
APPLICATION FILED DEC. 14, 1911.

1,067,528.

Patented July 15, 1913.



Witnesses:

*E. C. Payard*

*G. F. Chase*

Inventor:

Bernard C. Lauth

*By Dreyfus, LeGittine, Miles,  
Allison*

# UNITED STATES PATENT OFFICE.

BERNARD C. LAUTH, OF PITTSBURGH, PENNSYLVANIA, ASSIGNOR TO THOMAS S. BLAIR, JR., OF CHICAGO, ILLINOIS.

## METHOD FOR MAKING A MATERIAL HAVING THE GENERAL PROPERTIES OF WROUGHT-IRON.

BEST AVAILABLE COPY  
1,067,528.

Specification of Letters Patent.

Patented July 15, 1913.

Application filed December 14, 1911. Serial No. 665,655.

To all whom it may concern:

Be it known that I, BERNARD C. LAUTH, a citizen of the United States, residing at Pittsburgh, in the county of Allegheny and State of Pennsylvania, have invented a new and useful Improvement in Methods for Making a Material Having the General Properties of Wrought-Iron, of which the following is a specification.

10 My invention relates to an improved method for making a material having the general properties of wrought-iron. It involves in its practice a Bessemer converter of any form and a balling-furnace preferably, but not necessarily, of the type herein illustrated, Figure 1 being a diagrammatic representation of a Bessemer converter and Fig. 2 being a diagrammatic representation of a balling furnace of annular form and 15 adapted to revolve on its horizontal axis and to be oscillated upon a horizontal diameter for the purpose of discharging its contents.

I term the product of my process a material having the general properties of wrought-iron, because the leading authorities on iron and steel do not agree upon their definitions. One leading authority, for example, states in a general way, that the product of the puddling furnace is iron 20 and the product of a Bessemer converter is steel. The present product, resulting from a duplex process in which both a converter and a balling furnace are used, finds no place in this definition. It has, however, 25 the low carbon content and may, and preferably does have, the high slag content of wrought-iron, so that tested by any definition of the substance itself, apart from the process for making it, the substance is practically identical with ordinary wrought-iron.

There is an immense demand at the present time for wrought-iron providing the same can be supplied at anything approaching the cost of steel. The making of wrought-iron commercially is, however, essentially a hand-process, all efforts at mechanical puddling having failed for reasons which will hereinafter be pointed out. The 45 number of available trained puddlers is very limited and therefore the quantity of wrought-iron which can now be made at any price is limited, while the small units

in which the present puddling process must be worked and the very high labor cost, 55 make the price of even the small supply exceedingly high. One important result flowing from my invention is that the iron can be made mechanically and in large units so that the possible supply may be greatly increased and the cost diminished. It is also well known that at the present time the most desirable steel is made by the open-hearth process. There are in existence a very large number of Bessemer converters 65 which have either gone wholly out of use, or which are continued in operation, only because of the loss of investment which would be entailed if the Bessemer process were replaced by the better open-hearth process. 70

One principal object of the present invention is to enable these Bessemer converters to be profitably utilized in the manufacture of what is substantially wrought-iron, with but little additional outlay. In short, it is 75 believed that the use of the present invention will greatly increase the available supply of iron, while decreasing its cost, and will have an important reflex effect upon the average quality of the steel produced by reason of the fact that the present process will 80 make it possible for the Bessemer plants to continue in business without making steel.

In the ordinary puddling process, the molten impure or pig iron is stirred or agitated in the presence of iron oxid or ore, which is supplied as fettling lining in the puddling furnace. As the iron becomes purified and goes to nature it forms a ball to the surface of which pieces of the fettling 85 lining have a tendency to stick so as to be incorporated in the ball. The personal care of the puddler is required to prevent these pieces of ore from being picked up. If this personal care be removed, as in the case of 90 all mechanical puddling furnaces heretofore suggested, so much fettling gets worked into the ball as to produce such seriously detrimental effect as to have made all mechanical puddling devices wholly impractical, so that to-day wrought-iron is puddled by hand just as it always has been. The strength of the puddler is such that two hundred pounds is about the limit of the size of balls which can be made. Mechanical 100 puddling being thus made impracticable and

hand-puddling being limited to small units, furnish the reason for the small available supply of wrought-iron even at its present high cost.

I have discovered that molten pig iron can be blown in a Bessemer converter, of ordinary commercial form and preferably acid lined, such as that diagrammatically illustrated in Fig. 1, until sufficient iron oxid has been formed in the metal to oxidize whatever carbon may remain, and the product of this operation can be introduced into a suitable receptacle preferably a rotary or mechanical balling furnace of the type generally indicated in Fig. 2, which furnace has no fettling lining, and that in such furnace, under the influence of a reverberatory flame the iron oxid formed in the converter will react upon the remaining carbon, bringing the metal to nature expeditiously and cheaply, with the result that large balls can be quickly formed.

It is well understood in the Bessemer process that the carbon is oxidized before the iron, the oxidation of these materials overlapping, so that before all the carbon is oxidized, a considerable quantity of the iron is acted upon. In the ordinary use of the converter for making steel, iron oxid is a very objectionable product and therefore the treatment in the converter is usually stopped before any substantial oxidation of the iron occurs. The blast is never continued in steel making after the carbon reaches .05, and at that point some iron oxid is formed which must afterward be reduced by such deoxidizing agent as an excess of manganese or some aluminum. In the present process the blast is continued until enough iron oxid is formed to oxidize the remaining carbon. This point can readily be determined, in any given case, by the simplest chemical formula and the correct length of blow to produce the desired percentages of carbon and iron oxid can be made either by blowing a certain time after the "drop" or decrease in the carbon flame or by blowing a certain number of revolutions, as is now common practice.

In the blowing step, the slag-forming constituents are, in the main, eliminated, and should the remaining iron be balled alone, it would, it is thought, give too dry an iron. Therefore there is transferred to the balling furnace of Fig. 2, with the iron, a suitable quantity of slag. This preliminary separation of iron and slag has the advantage that the slag can be modified in any way desired to produce the best wrought-iron under all the conditions, and a wholly new slag may be made if desired for special purposes. However, in most cases the slag is the converter slag without modification. The balling furnace has a refractory lining of the same general character (acid

or basic) as the slag, and therefore usually of the same character as the lining of the converter used.

The lining is made free from separable particles which, like the fettling of a puddling furnace, may be worked into the ball.

The balling furnace with its charge of iron and slag is rotated to keep the charge in motion, and the iron oxid reacts on the carbon, bringing the metal to nature. As successive particles reach this point they unite until a ball of some size is formed which rolls around the balling furnace, picking up from the bath of slag and molten iron successive particles as they go to nature, until at length all the metal is incorporated in the ball. The furnace is then dumped, or the ball otherwise removed, any iron oxid not reduced in oxidizing the carbon remaining in the slag. With the nice methods now well known for predetermining the constituents of the product of the Bessemer converter, it is possible to balance the carbon and iron oxid accurately so that the iron oxidized in the converter will be almost wholly reduced in the balling furnace, to the end that but slight waste of iron will occur.

It is evident that the final or balling step is wholly mechanical and can be worked on large as well as on small charges, the only limit being the size of balls that may be conveniently handled in rolling processes to follow. I contemplate making balls of about the weight of ingots now being used in any given plant, so that there need be no substantial change in rolling methods. The manufacture of finished iron products can thus be substituted for that of Bessemer steel products upon the installation of the balling furnaces in suitable numbers to handle the product of the converters and of one or more squeezers to reduce the balls to proper size for the first passes of the rolls.

I realize that the foregoing process is subject to considerable variation in detail and I do not therefore intend to be limited to the specific embodiment shown, except as pointed out in the following claims, in which my intention is to claim all the novelty in the process as broadly as is permitted by the state of the art.

What I claim as new and desire to secure by Letters Patent is—

1. The method which consists in blowing molten impure iron according to the Bessemer process until the carbon is substantially oxidized and iron oxid is formed in sufficient quantity to oxidize the remaining carbon, and thereupon transferring the molten metal to a receptacle and agitating it until the iron oxid oxidizes the carbon and the metal goes to nature.

2. The method which consists in blowing molten impure iron according to the

Bessemer process until the carbon is substantially oxidized and iron oxid is formed in sufficient quantity to oxidize the remaining carbon, and thereupon transferring the molten metal to a receptacle free from fettling and agitating it until the iron oxid oxidizes the carbon and the metal goes to nature.

3. The method which consists in blowing molten impure iron according to the Bessemer process until the carbon is substantially oxidized and iron oxid is formed in sufficient quantity to oxidize the remaining carbon, and thereupon transferring the molten metal with a quantity of slag to a receptacle and agitating it until the iron oxid oxidizes the carbon and the metal goes to nature.

4. The method which consists in blowing molten impure iron according to the Bessemer process until the carbon is substantially oxidized and iron oxid is formed in sufficient quantity to oxidize the remaining carbon, and thereupon transferring the molten metal, with a quantity of the slag formed in the Bessemer operation, to a receptacle and agitating it until the iron oxid oxidizes the carbon and the metal goes to nature.

5. The method which consists in blowing molten impure iron according to the Bessemer process until the carbon is substantially oxidized and iron oxid is formed in sufficient quantity to oxidize the remaining car-

bon, and thereupon transferring the molten metal, with a quantity of slag, to a receptacle having a lining of the same acid or basic character as the slag, and agitating it until the iron oxid oxidizes the carbon and the metal goes to nature.

6. The method which consists in blowing molten impure iron according to the Bessemer process until the carbon is substantially oxidized and iron oxid is formed in sufficient quantity to oxidize the remaining carbon, and thereupon transferring the molten metal, and a quantity of the slag formed in the Bessemer operation, to a receptacle having a lining of the same acid or basic character as the converter and there agitating it until the iron oxid oxidizes the carbon and the metal goes to nature.

7. The method which consists in blowing molten impure iron according to the acid Bessemer process until the carbon is substantially oxidized and iron oxid is formed in sufficient quantity to oxidize the remaining carbon, and thereupon transferring the molten metal, and some of the Bessemer slag, to an acid lined receptacle and agitating it until the iron oxid oxidizes the carbon and the metal goes to nature.

BERNARD C. LAUTH.

In presence of—

RUSSELL WILES,  
DUDLEY BROWNE.

Copies of this patent may be obtained for five cents each, by addressing the "Commissioner of Patents, Washington, D. C."